



US009529288B1

(12) **United States Patent**  
Sugawara et al.

(10) **Patent No.:** US 9,529,288 B1  
(45) **Date of Patent:** Dec. 27, 2016

(54) **ELECTROSTATIC CHARGE IMAGE DEVELOPING TONER, ELECTROSTATIC CHARGE IMAGE DEVELOPER, AND TONER CARTRIDGE**

(71) Applicant: **FUJI XEROX CO., LTD.**, Tokyo (JP)

(72) Inventors: **Atsushi Sugawara**, Kanagawa (JP); **Kana Yoshida**, Kanagawa (JP); **Tsuyoshi Murakami**, Kanagawa (JP); **Yukiaki Nakamura**, Kanagawa (JP)

(73) Assignee: **FUJI XEROX CO., LTD.**, Tokyo (JP)

(\*) Notice: Subject to any disclaimer, the term of this patent is extended or adjusted under 35 U.S.C. 154(b) by 0 days.

(21) Appl. No.: **15/007,911**

(22) Filed: **Jan. 27, 2016**

(30) **Foreign Application Priority Data**

Aug. 25, 2015 (JP) ..... 2015-165797

(51) **Int. Cl.**

**G03G 9/093** (2006.01)  
**G03G 9/08** (2006.01)  
**G03G 15/08** (2006.01)  
**G03G 9/087** (2006.01)

(52) **U.S. Cl.**

CPC ..... **G03G 9/08** (2013.01); **G03G 9/08755** (2013.01); **G03G 15/0865** (2013.01)

(58) **Field of Classification Search**  
CPC ..... G03G 9/09307; G03G 9/09342  
See application file for complete search history.

(56) **References Cited**

U.S. PATENT DOCUMENTS

2009/0047595 A1 \* 2/2009 McDougall ..... G03G 9/0804  
430/137.14  
2011/0059394 A1 3/2011 Mutoh et al.

FOREIGN PATENT DOCUMENTS

JP 2011-081344 A 4/2011  
JP 2013-003196 A 1/2013  
JP 2014-209188 A 11/2014

\* cited by examiner

Primary Examiner — Hoa V Le

(74) Attorney, Agent, or Firm — Oliff PLC

(57) **ABSTRACT**

An electrostatic charge image developing toner includes a toner particle containing a binder resin, a release agent, and an inorganic mineral, wherein 80% or more of the entire release agent is present in a portion within 400 nm from the surface of the toner particle and 80% or more of the entire inorganic mineral is present in a portion within 400 nm from the surface of the toner particle.

**9 Claims, 3 Drawing Sheets**



FIG. 1



FIG. 2



FIG. 3



**ELECTROSTATIC CHARGE IMAGE  
DEVELOPING TONER, ELECTROSTATIC  
CHARGE IMAGE DEVELOPER, AND TONER  
CARTRIDGE**

**CROSS-REFERENCE TO RELATED  
APPLICATIONS**

This application is based on and claims priority under 35 USC 119 from Japanese Patent Application No. 2015-165797 filed Aug. 25, 2015.

**BACKGROUND**

1. Technical Field

The present invention relates to an electrostatic charge image developing toner, an electrostatic charge image developer, and a toner cartridge.

2. Related Art

A method of visualizing image information through electrophotography is currently used in various fields. In electrophotography, an electrostatic charge image is formed on a surface of an image holding member as image information through charging and electrostatic charge image formation. A toner image is formed on the surface of the image holding member using a developer containing a toner, and the toner image is transferred to a recording medium, and then the toner image is fixed onto a surface of the recording medium. The image information is visualized as an image through these processes.

**SUMMARY**

According to an aspect of the invention, there is provided an electrostatic charge image developing toner including: a toner particle containing a binder resin, a release agent, and an inorganic mineral, wherein 80% or more of the entire release agent is present in a portion within 400 nm from a surface of the toner particle, and 80% or more of the entire inorganic mineral is present in a portion within 400 nm from the surface of the toner particle.

**BRIEF DESCRIPTION OF THE DRAWINGS**

Exemplary embodiments of the present invention will be described in detail based on the following figures, wherein:

FIG. 1 is a diagram showing a cross section of a toner particle according to the exemplary embodiment;

FIG. 2 is a schematic configuration diagram showing an image forming apparatus according to the exemplary embodiment; and

FIG. 3 is a schematic configuration diagram showing an example of a process cartridge according to the exemplary embodiment.

**DETAILED DESCRIPTION**

Hereinafter, exemplary embodiments which are examples of the invention will be described in detail.

**Electrostatic Charge Image Developing Toner**

An electrostatic charge image developing toner according to the exemplary embodiment (hereinafter, also referred to as a "toner") contains a toner particle having a binder resin, a release agent, and an inorganic mineral.

In the toner particle, 80% or more of the entire release agent is present in a portion within 400 nm from the surface of the toner particle (hereinafter, a percentage of the release agent which is present in a portion within 400 nm from the surface of the toner particle is also referred to as a "presence ratio (400 nm) of the release agent").

In addition, 80% or more of the entire inorganic mineral is present in a portion within 400 nm from the surface of the toner particle (hereinafter, a percentage of the inorganic mineral present in a portion within 400 nm from the surface of the toner particle is also referred to as a "presence ratio (400 nm) of the inorganic mineral").

According to the configuration described above, the toner according to the exemplary embodiment prevents occurrence of image deletion. The reason therefor is not clear, but the following are assumed.

A toner in which a release agent is arranged in a surface portion of a toner particle (for example, a range within 400 nm from the surface of the toner particle) is excellent in maintaining peeling properties of a fixed image from a fixing member. However, since the release agent is arranged in the surface portion of the toner particle, abrasion occurs in the surface portion of the toner particle by stirring in a developing unit (developing device), and the release agent is easily exposed from the surface of the toner particle. Particularly, when an electrostatic charge image developer (hereinafter, also referred to as a "developer") is a two-component developer, abrasion more easily occurs in the surface portion of the toner particle due to friction with a carrier, and the release agent is more easily exposed on the surface of the toner particle. Accordingly, the solidification of the toner may occur in the developing device due to aggregation of the toner particles on which the release agents are exposed. If an image is formed in a state where the toner is solidified, image deletion may easily occur in an image to be formed. It is found that this phenomenon easily occurs when a solid image having high image density (for example, image density equal to or greater than 80%) is formed after continuously forming images having low image density (for example, image density equal to or smaller than 5%), and more easily occurs particularly when an image is formed in a high temperature and high humidity environment (for example, temperature of 32°C. and humidity of 90 RH %).

Toner is agitated in the developing device and friction occurs on the surface of the toner particle. In a case of forming an image having low image density, an amount of toner transferred to the image holding member is small, and the same toner particles are continuously agitated in the developing device, and therefore, friction with the surface of the toner particle more easily occurs. It is considered that while images having low image density are continuously formed, the release agent is exposed on the surface of the toner particle due to abrasion occurring in the surface portion of the toner particle, the toner particles on which the release agents are exposed are aggregated and solidification of the toner occurs. This phenomenon more easily occurs, when the developer is a two-component developer. As a result, when a solid image having high image density is formed after continuously forming images having low image density, image deletion easily occurs.

With respect to this, the toner according to the exemplary embodiment includes, as described above, a toner particle in which the presence ratio of the release agent is equal to or greater than 80% and the presence ratio (400 nm) of the inorganic mineral is equal to or greater than 80%.

When the presence ratio (400 nm) of the inorganic mineral is equal to or greater than 80%, strength of the surface of the toner particle is improved due to a filler effect of the inorganic mineral. Accordingly, for example, even when a mechanical load is applied to the toner particles due to friction with the surface of the toner particles in the developing device, abrasion to the surface portion of the toner particle is prevented, and accordingly, the release agent present in the surface portion of the toner particles is prevented from being exposed on the surface of the toner particle. As a result, since solidification of the toner occurring in the developing device due to aggregation of the toner particles on which the release agents are exposed is prevented, the occurrence of image deletion is prevented, even when an image having high image density is formed after continuously forming images having low image density in a high temperature and high humidity environment.

Based on the above, it is assumed that the toner according to the exemplary embodiment prevents occurrence of image deletion with the configurations described above.

Hereinafter, the toner according to the exemplary embodiment will be described in detail.

The toner according to the exemplary embodiment contains a toner particle, and if necessary, an external additive.

#### Toner Particles

The toner particle according to the exemplary embodiment includes a specific release agent domain, and for example, contains a binder resin, a release agent, if necessary, a colorant and other additives.

#### Binder Resin

Examples of the binder resins include a vinyl resin formed of a homopolymer of monomers such as styrenes (for example, styrene, p-chlorostyrene,  $\alpha$ -methyl styrene, or the like), (meth)acrylic esters (for example, methyl acrylate, ethyl acrylate, n-propyl acrylate, n-butyl acrylate, lauryl acrylate, 2-ethylhexyl acrylate, methyl methacrylate, ethyl methacrylate, n-propyl methacrylate, lauryl methacrylate, 2-ethylhexyl methacrylate, or the like), ethylenic unsaturated nitriles (for example, acrylonitrile, methacrylonitrile, or the like), vinyl ethers (for example, vinyl methyl ether, vinyl isobutyl ether, or the like), vinyl ketones (for example, vinyl methyl ketone, vinyl ethyl ketone, vinyl isopropenyl ketone, or the like), olefins (for example, ethylene, propylene, butadiene, or the like), or a copolymer obtained by combining two or more kinds of these monomers.

Examples of the binder resin include a non-vinyl resin such as an epoxy resin, a polyester resin, a polyurethane resin, a polyamide resin, a cellulose resin, a polyether resin, and a modified rosin, a mixture of these and a vinyl resin, or a graft polymer obtained by polymerizing a vinyl monomer in the presence thereof.

These binder resins may be used alone or in combination with two or more kinds thereof.

A polyester resin is suitable as the binder resin.

As the polyester resin, a well-known polyester resin is used, for example.

As the polyester resin, a well-known polyester resin is used, for example.

Examples of the polyester resin include condensation polymers of polyvalent carboxylic acids and polyols. A commercially available product or a synthesized product may be used as the polyester resin.

Examples of the polyvalent carboxylic acid include aliphatic dicarboxylic acids (e.g., oxalic acid, malonic acid, maleic acid, fumaric acid, citraconic acid, itaconic acid, glutaconic acid, succinic acid, alkenyl succinic acid, adipic acid, and sebamic acid), alicyclic dicarboxylic acids (e.g.,

cyclohexanedicarboxylic acid), aromatic dicarboxylic acids (e.g., terephthalic acid, isophthalic acid, phthalic acid, and naphthalenedicarboxylic acid), anhydrides thereof, or lower alkyl esters (having, for example, from 1 to 5 carbon atoms) thereof. Among these, for example, aromatic dicarboxylic acids are preferably used as the polyvalent carboxylic acid.

As the polyvalent carboxylic acid, a tri- or higher-valent carboxylic acid employing a crosslinked structure or a branched structure may be used in combination together with a dicarboxylic acid. Examples of the tri- or higher-valent carboxylic acid include trimellitic acid, pyromellitic acid, anhydrides thereof, or lower alkyl esters (having, for example, from 1 to 5 carbon atoms) thereof.

The polyvalent carboxylic acids may be used alone or in combination of two or more kinds thereof.

Examples of the polyol include aliphatic diols (e.g., ethylene glycol, diethylene glycol, triethylene glycol, propylene glycol, butanediol, hexanediol, and neopentyl glycol), alicyclic diols (e.g., cyclohexanediol, cyclohexanedimethanol, and hydrogenated bisphenol A), and aromatic diols (e.g., ethylene oxide adduct of bisphenol A and propylene oxide adduct of bisphenol A). Among these, for example, aromatic diols and alicyclic diols are preferably used, and aromatic diols are more preferably used as the polyol.

As the polyol, a tri- or higher-valent polyol employing a crosslinked structure or a branched structure may be used in combination together with a diol. Examples of the tri- or higher-valent polyol include glycerin, trimethylolpropane, and pentaerythritol.

The polyols may be used alone or in combination of two or more kinds thereof.

The glass transition temperature (Tg) of the polyester resin is preferably from 50° C. to 80° C., and more preferably from 50° C. to 65° C.

The glass transition temperature is obtained by a DSC curve which is obtained by a differential scanning calorimetry (DSC), and more specifically, is obtained by "Extrapolating Glass Transition Starting Temperature" disclosed in a method for obtaining the glass transition temperature of "Testing Methods for Transition Temperatures of Plastics" in JIS K-7121-1987.

A weight-average molecular weight (Mw) of the polyester resin is preferably from 5,000 to 1,000,000, and more preferably from 7,000 to 500,000.

The number-average molecular weight (Mn) of the polyester resin is preferably from 2,000 to 100,000.

The molecular weight distribution Mw/Mn of the polyester resin is preferably from 1.5 to 100, and more preferably from 2 to 60.

The weight-average molecular weight and the number-average molecular weight are measured by gel permeation chromatography (GPC). The molecular weight measurement by GPC is performed with a THF solvent using HLC-8120 GPC, which is GPC manufactured by Tosoh Corporation as a measurement device by using TSKGEL Super HM-M (15 cm), which is a column manufactured by Tosoh Corporation. The weight-average molecular weight and the number-average molecular weight are calculated using a calibration curve of molecular weight created with a monodisperse polystyrene standard sample from results of this measurement.

The polyester resin is obtained with a well-known preparing method. Specific examples thereof include a method of conducting a reaction at a polymerization temperature set to 180° C. to 230° C., if necessary, under reduced pressure

in the reaction system, while removing water or an alcohol generated during condensation.

When monomers of the raw materials are not dissolved or compatibilized under a reaction temperature, a high-boiling-point solvent may be added as a solubilizing agent to dissolve the monomers. In this case, a polycondensation reaction is conducted while distilling away the solubilizing agent. When a monomer having poor compatibility is present in a copolymerization reaction, the monomer having poor compatibility and an acid or an alcohol to be polycondensed with the monomer may be previously condensed and then polycondensed with the major component.

The content of the binder resin is preferably from 40% by weight to 95% by weight, more preferably from 50% by weight to 90% by weight, and even more preferably from 60% by weight to 85% by weight, with respect to the entire toner particles.

#### Release Agent

Examples of the release agent include hydrocarbon waxes; natural waxes such as carnauba wax, rice wax, and candelilla wax; synthetic or mineral/petroleum waxes such as montan wax and Fischer Tropsch Wax; and ester waxes such as fatty acid esters and montanic acid esters. The release agent is not limited thereto.

Among these, hydrocarbon waxes are preferable, because a shape of the release domain easily satisfy Condition (1) to Condition (4) described above.

The melting temperature of the release agent is preferably from 50° C. to 110° C., and more preferably from 60° C. to 100° C.

Further, the melting temperature is determined from a DSC curve obtained by differential scanning calorimetry (DSC), using the "melting peak temperature" described in the method of determining a melting temperature in the "Testing Methods for Transition Temperatures of Plastics" in JIS K-7121-1987.

The content of the release agent is, for example, preferably from 1% by weight to 20% by weight, and more preferably from 5% by weight to 15% by weight, with respect to the entire toner particles.

#### Inorganic Mineral

The inorganic mineral is not particularly limited, but in order to prevent occurrence of image deletion, a silicate mineral may be used, and a clay mineral having a layered structure (hereinafter, also referred to as a "layered clay mineral") is preferably used. When the inorganic mineral is a layered clay mineral, 80% or more of the entire inorganic mineral is easily present in a portion within 400 nm from the surface of the toner particle and strength of the toner particle is easily improved due to a filler effect.

As the layered clay mineral, a type having great cation exchange capacity may be selected, in order to prevent occurrence of image deletion. Since the layered clay mineral having great cation exchange capacity is easily bonded with a carboxylic group present in the surface of the binder resin in the toner particle and anions such as sulfonic acid ions of a surfactant adsorbed to the binder resin, for example, the strength of the surface of the toner particle is easily improved.

Specific examples of the layered clay mineral include kaolinite (kaolinite, halloysite, or the like), smectite (montmorillonite, beidellite, saponite, hectorite, stevensite, or the like). Further, illite, mica, vermiculite, talc, pyrophyllite, chlorite, or the like is used. Among the layered clay minerals, smectite and kaolinite having particularly greater cation exchange capacity are preferable and among these, smectite is more preferable.

A volume average particle diameter of the inorganic mineral may be from 0.2 µm to 1.5 µm and is preferably from 0.2 µm to 1.0 µm, in order that 80% or more of the entire inorganic mineral is easily present in a portion within 400 nm from the surface of the toner particle.

A method of measuring the volume average particle diameter of the inorganic mineral in the toner particle is as follows. A solvent, which may dissolve only a resin component of the toner without dissolving the inorganic mineral, and a toner are mixed with each other and stirred, so that the resin component of the toner is dissolved in the solvent, and then, solid-liquid separation is performed to obtain an inorganic mineral (herein, when an external additive is attached to the surface of the toner particle, the external additive attached to the surface of the toner particle is removed). Regarding the separated inorganic mineral, cumulative distributions by volume are drawn from the side of the smallest diameter with respect to particle size ranges (channels) divided based on the particle size distribution measured by a particle size distribution measuring device (COULTER MULTISIZER II (manufactured by Beckman Coulter K.K.)), and the particle diameter when the cumulative percentage becomes 50% is defined as that corresponding to a volume average particle diameter. The volume average particle diameter is a sphere equivalent diameter.

The content of the inorganic mineral may be from 1% by weight to 10% by weight and is preferably 1% by weight to 5% by weight with respect to the entire toner particles, for example, in order to prevent occurrence of image deletion.

The weight ratio of the inorganic mineral to the release agent may be in a range of from 1:1 to 1:15.

In the toner of the exemplary embodiment, the "inorganic mineral present in a portion within 400 nm from the surface of the toner particle" is contained in the toner particle and does not include a so-called externally added inorganic mineral.

#### Colorant

Examples of the colorant include various pigments such as carbon black, chrome yellow, Hansa yellow, benzidine yellow, threne yellow, quinoline yellow, pigment yellow, permanent orange GTR, pyrazolone orange, vulcan orange, watchung red, permanent red, brilliant carmine 3B, brilliant carmine 6B, DuPont oil red, pyrazolone red, lithol red, Rhodamine B Lake, Lake Red C, pigment red, rose bengal, aniline blue, ultramarine blue, calco oil blue, methylene blue chloride, phthalocyanine blue, pigment blue, phthalocyanine green, and malachite green oxalate, and various dyes such as acridine dyes, xanthene dyes, azo dyes, benzoquinone dyes, azine dyes, anthraquinone dyes, thioindigo dyes, dioxadine dyes, thiazine dyes, azomethine dyes, indigo dyes, phthalocyanine dyes, aniline black dyes, polymethine dyes, triphenylmethane dyes, diphenylmethane dyes, and thiazole dyes.

The colorants may be used alone or in combination of two or more kinds thereof.

If necessary, the colorant may be surface-treated or used in combination with a dispersing agent. Plural kinds of colorants may be used in combination.

The content of the colorant is, for example, preferably from 1% by weight to 30% by weight, and more preferably from 3% by weight to 15% by weight with respect to the entirety of the toner particles.

#### Other Additives

Examples of other additives include known additives such as a magnetic material, a charge-controlling agent, and an inorganic powder. The toner particles contain these additives as internal additives.

## Characteristics of Toner Particle

The toner particle may be toner particle having a single-layer structure, or toner particles having a so-called core/shell structure composed of a core (core particle) and a coating layer (shell layer) coated on the core.

When the toner particle includes a core particle and a shell layer coated on the core particle, the shell layer may preferably contain the release agent and the inorganic mineral. When the shell layer may contain the release agent and the inorganic mineral, the release agent and the inorganic mineral are present in the surface portion of the toner particle, and accordingly, the release agent is prevented from being exposed on the surface of the toner particle and abrasion to the surface of the toner particle is easily prevented.

The toner particle may include a core particle, a first shell layer coated on the core particle, and a second shell layer coated on the first shell layer.

When the toner particle includes the core particle, the first shell layer coated on the core particle, and the second shell layer coated on the first shell layer, it is preferable that the first shell layer may contain the release agent and the second shell layer may contain the inorganic mineral.

When the first shell layer contains the release agent, the release agent is easily present in the surface portion of the toner particle and the release agent more easily bleeds to the surface of the toner particle at the time of toner fixation. The second shell layer coated on the first shell layer is present and the inorganic mineral is present in the second shell layer. Accordingly, the inorganic mineral is present on the surface side with respect to the release agent, and accordingly, the release agent is further prevented from being exposed on the surface of the toner particle and abrasion to the surface of the toner particle is further easily prevented. The inorganic mineral may be contained in both layers of the first shell layer and the second shell layer coated thereon.

The volume average particle size (D50v) of the toner particles is preferably from 2  $\mu\text{m}$  to 10  $\mu\text{m}$ , and more preferably from 4  $\mu\text{m}$  to 8  $\mu\text{m}$ .

Various average particle sizes and various particle size distribution indices of the toner particles are measured using a COULTER MULTISIZER II (manufactured by Beckman Coulter, Inc.) and ISOTON-II (manufactured by Beckman Coulter, Inc.) as an electrolyte.

In the measurement, from 0.5 mg to 50 mg of a measurement sample is added to 2 ml of a 5% aqueous solution of surfactant (preferably sodium alkylbenzene sulfonate) as a dispersing agent. The obtained material is added to 100 ml to 150 ml of the electrolyte.

The electrolyte in which the sample is suspended is subjected to a dispersion treatment using an ultrasonic disperser for 1 minute, and a particle size distribution of particles having a particle size of 2  $\mu\text{m}$  to 60  $\mu\text{m}$  is measured by a COULTER MULTISIZER II using an aperture having an aperture size of 100  $\mu\text{m}$ . 50,000 particles are sampled.

Cumulative distributions by volume and by number are drawn from the side of the smallest size with respect to particle size ranges (channels) separated based on the measured particle size distribution. The particle size when the cumulative percentage becomes 16% is defined as that corresponding to a volume average particle size D16v and a number-average particle size D16p, while the particle size when the cumulative percentage becomes 50% is defined as that corresponding to a volume average particle size D50v and a number-average particle size D50p. Furthermore, the particle size when the cumulative percentage becomes 84%

is defined as that corresponding to a volume average particle size D84v and a number-average particle size D84p.

Using these, a volume average particle size distribution index (GSDv) is calculated as  $(D84v/D16v)^{1/2}$ , while a number-average particle size distribution index (GSDp) is calculated as  $(D84p/D16p)^{1/2}$ .

The shape factor SF1 of the toner particles is preferably from 110 to 150, and more preferably from 120 to 140.

The shape factor SF1 is obtained through the following expression.

$$SF1 = (ML^2/A) \times (\pi/4) \times 100$$

Expression:

In the foregoing expression, ML represents an absolute maximum length of a toner, and A represents a projected area of a toner.

Specifically, the shape factor SF1 is numerically converted mainly by analyzing a microscopic image or a scanning electron microscopic (SEM) image by using of an image analyzer, and is calculated as follows. That is, an optical microscopic image of particles scattered on a surface of a glass slide is input to an image analyzer LUZEX through a video camera to obtain maximum lengths and projected areas of 100 particles, values of SF1 are calculated through the foregoing expression, and an average value thereof is obtained.

In the toner particle of the toner according to the exemplary embodiment, the presence ratio (400 nm) of the release agent is equal to or greater than 80%. The presence ratio (400 nm) of the release agent is preferably from 85% to 100% and more preferably from 90% to 100%. The presence ratio (400 nm) of the release agent is preferably in the range described above, in a viewpoint of peeling properties of a fixed image from the fixing member.

As a method of controlling the presence ratio (400 nm) of the release agent to be equal to or greater than 80%, a method of setting the toner particle to have a core/shell structure and using a release agent when forming a shell is used, for example.

In the toner particle of the toner according to the exemplary embodiment, the presence ratio (400 nm) of the inorganic mineral (that is, percentage of the inorganic mineral present in a portion within 400 nm from the surface of the toner particle) is equal to or greater than 80%. The presence ratio of the inorganic mineral is preferably from 85% to 100% and more preferably from 90% to 100%, in order to further prevent image deletion.

The percentage of the inorganic mineral present in a portion within 300 nm from the surface of the toner particle (hereinafter, also referred to as the presence ratio (300 nm) of the inorganic mineral") is preferably equal to or greater than 80%, more preferably from 85% to 100%, and even more preferably from 90% to 100%. The percentage of the inorganic mineral present in a portion within 225 nm from the surface of the toner particle (hereinafter, also referred to as the presence ratio (225 nm) of the inorganic mineral") is preferably equal to or greater than 80%, more preferably from 85% to 100%, and even more preferably from 90% to 100%.

Meanwhile, it is preferable that the percentage of the release agent present in a portion within 300 nm from the surface of the toner particle is equal to or smaller than 20% (more preferably from 0% to 10% and even more preferably 0% to 5%). Hereinafter, the percentage of the release agent present in a portion within 300 nm from the surface of the toner particle is also referred to as a "presence ratio (300 nm) of the release agent".

In order to further prevent image deletion, it is particularly preferable that a larger amount of the inorganic mineral is present on a surface side of the toner particle than an amount of the release agent present in a portion within 400 nm from the surface of the toner particle.

Since a larger amount of the inorganic mineral is present on a surface side of the toner particle than an amount of the release agent present in a portion within 400 nm from the surface of the toner particle, the strength of the toner particle is more easily improved.

From such a viewpoint, it is preferable that, in the toner of the exemplary embodiment, 20% or less (more preferably 0% to 10% and even more preferably 0% to 5%) of the entire release agent is present in a portion within 300 nm from the surface of the toner particle and 80% or more (more preferably 85% to 100% and even more preferably 90% to 100%) of the entire inorganic mineral is present in a portion within 300 nm from the surface of the toner particle.

As a method of controlling the presence ratio (400 nm) of the inorganic mineral to be equal to or greater than 80%, a method of setting the toner particle to have a core/shell structure and using the inorganic mineral when forming a shell is used, for example. As a method of controlling the presence ratio (300 nm) of the inorganic mineral (or presence ratio (225 nm) of the inorganic mineral) to be equal to or greater than 80%, a method of setting the toner particle to have a core/first shell/second shell structure and using the inorganic mineral when forming a second shell is used, for example.

As a method of controlling the presence ratio (300 nm) of the release agent to be equal to or less than 20%, a method of setting the toner particle to have a core/first shell/second shell structure and using the release agent when forming a first shell and not using the release agent when forming a second shell is used, for example.

In the toner particle of the toner according to the exemplary embodiment, it is preferable that the release agent domain satisfying Condition (1) to Condition (4) described below (hereinafter, the release agent domain satisfying Condition (1) to Condition (4) described below may be referred to as a "specific release agent domain") is formed, from a viewpoint of peeling properties of a fixed image from the fixing member.

Condition (1): a length of the release agent domain in a long axis direction is from 300 nm to 1200 nm

Condition (2): a ratio between a length of the release agent domain in a long axis direction and a length thereof in a short axis direction (length in a long axis direction/length in a short axis direction) is from 3.0 to 15.0

Condition (3): an angle formed by a tangent line passing a tangent point of a circumference of a circle centered at a centroid of the release agent domain and inscribed in an outer edge of the toner particle and the outer edge, and a line which passes the centroid of the release agent domain and extends in the long axis direction of the release agent domain is from 0° to 45°

Condition (4): a ratio between a circle equivalent diameter of the toner particle and a distance A between the centroid of the release agent domain and the tangent point (distance A/circle equivalent diameter) is from 0.03 to 0.25

It is assumed that the release agent domain satisfying Condition (1) to Condition (4) described above exhibits the following effects.

When the release agent domain satisfies Condition (1), it is easy to ensure an amount of the release agent which is necessary for causing the release agent to bleed from the release agent domain to exhibit releasing properties.

When the release agent domain satisfies Condition (2), a contact area of the release agent domain elongated in the long axis direction with a sheet at the time of fixing is increased and it is easy to increase an amount of the release agent.

When the release agent domain satisfies Condition (3), the contact area with the sheet is further increased at the time of fixing, and accordingly, the release agent effectively easily bleeds out at the time of fixing.

When the release agent domain satisfies Condition (4), the release agent domain is arranged in the surface portion of the toner particle, and accordingly, the release agent bled from the release agent domain easily bleeds out to the external portion of the toner particle.

Herein, a relationship between the toner particle and the release agent domain will be described with reference to the drawing.

FIG. 1 is a diagram showing a cross section of the toner particle according to the exemplary embodiment. In FIG. 1, a toner particle 100 includes plural release agent domains 102. A circle which is centered at a centroid B of the release agent domain 102 and inscribed in an outer edge of the toner particle 100 is shown as a circle C in FIG. 1. A radius of the circle C, that is, a distance between a tangent point at which the outer edge of the toner particle 100 and the circle C are inscribed, and the centroid B is set as a distance A. A line which passes the centroid B of the release agent domain 102 and extends in the long axis direction of the release agent domain 102 is set as a line D. A tangent line which passes a tangent point of the circumference of the circle C and the outer edge of the toner particle 100 is set as a line E. An angle (acute angle) formed by the line D and the line E is set as θ. When θ is 0°, it shows that the line D and the line E does not intersect with each other.

In the exemplary embodiment, the presence ratio of the release agent contained in the toner particle and the presence ratio of the inorganic mineral contained in the toner particle are calculated by observing the cross section of the toner particle and the observation of the specific release agent domain contained in the toner particle is performed using the cross section of the toner particle.

The cross section of the toner particle is, for example, checked by a method of observing the cross section of the toner particle using a transmission electron microscope (TEM) or a method of dying the cross section of the toner particle with ruthenium tetroxide and observing the cross section thereof using a scanning electron microscope (SEM). In order to more clearly observe the release agent domain of the cross section of the toner, a method of observing the cross section thereof with a scanning electron microscope is preferably used. As the scanning electron microscope, any scanning electron microscope which is well known by a person skilled in the art may be used, and for example, SU8020 manufactured by Hitachi High-Technologies Corporation or JSM-7500F manufactured by JEOL, Ltd. is used.

The preparation of a measurement sample for observing the cross section of the toner particle is performed with the following procedure. A toner particle to be measured is embedded in an epoxy resin, and then the epoxy resin is cured. The cured substance is cut into a thin section with a microtome including a diamond blade (for example, ULTRACUT UCT manufactured by Leica), thereby obtaining a measurement sample in which a cross section of the toner is exposed.

In a case where an external additive is attached to the surface of the toner particle when obtaining the measure-

## 11

ment sample, the external additive attached to the surface of the toner particle is removed. Specifically, several droplets of a surfactant such as contamination (manufactured by Wako Pure Chemical Industries, Ltd.) is added to ion exchange water, the toner is added thereto and dispersed, the resultant material is irradiated with ultrasonic waves for 1 minute to 5 minutes, and thereby the external additive attached to the surface of the toner particle is removed. After that, a dispersion of the toner particle passes through filter paper and subjected to rinse cleaning, and the toner particles on the filter paper are dried to obtain toner particles for preparing the measurement sample.

A method of measuring the presence ratio (400 nm) of the release agent and the presence ratio (300 nm) of the release agent will be described.

The thin measurement sample prepared as described above in which a cross section of the toner is exposed is dyed with ruthenium tetroxide, an SEM image of the cross section of the toner particle is obtained with a scanning electron microscope and the cross section of the toner particle is observed. With the method, each component in the cross section of the toner article is identified by a difference in shading caused by the degree of dyeing, and the release agent is observed.

In the SEM image, the cross section of the toner particle having a maximum length which is 85% or more of a volume average particle diameter of the toner particles is selected, the domain of the dyed release agent is observed, the area of the release agent of the entire toner particle and the area of the release agent present in an area within 400 nm (or within 300 nm) from the surface of the toner particle are determined, and a ratio of both areas (area of the release agent present in an area within 400 nm (or within 300 nm) from the surface of the toner particle/area of the release agent of the entire toner particle) is calculated. This calculation is performed for 100 toner particles which are arbitrarily selected, and an average value thereof is set as the presence ratio of the release agent.

The reason for selecting the cross section of the toner particle having a maximum length which is 85% or more of a volume average particle diameter of the toner particles is as follows. Since the toner is a three-dimensional shape and the SEM image is a cross section, the end portion may be cut and the cross section of the end portion does not reflect the domain of the release agent of the toner.

The presence ratio (400 nm) of the inorganic mineral and the presence ratio (300 nm) of the inorganic mineral will be described.

An SEM image of the measurement sample prepared as described above in which a cross section of the toner is exposed is obtained. Element analysis of the measurement sample of the cross section of the toner particle is performed using an energy dispersive X-ray analyzer (SEM-EDX device) attached to a scanning electron microscope, and each presence ratio of each inorganic mineral is measured by a mapping process.

Regarding each presence ratio of the inorganic mineral, an area of the inorganic mineral of the entire toner particle and an area of the inorganic mineral present in an area within 400 nm (within or 300 nm) from the surface of the toner particle are determined, and a ratio of both areas (area of the inorganic mineral present in an area within 400 nm (or within 300 nm) from the surface of the toner particle/area of the inorganic mineral of the entire toner particle) is calculated. This calculation is performed for 100 toner particles which are arbitrarily selected, and an average value thereof is set as the presence ratio of each inorganic mineral.

## 12

The observation of the cross section of the specific release agent domain will be described.

A method of determining an angle formed by a tangent line passing a tangent point of a circumference of a circle centered at a centroid of the release agent domain and inscribed in an outer edge of the toner particle and the outer edge, and a line which passes the centroid of the release agent domain and extends in the long axis direction of the release agent domain will be described.

10 An image is recorded at magnification which allows a cross section of one toner particle to come in sight. Image analysis for the recorded image is performed under a condition of 0.010000  $\mu\text{m}/\text{pixel}$  by using image analysis software (WINROOF manufactured by MITANI Corporation).

15 An image of the cross section of the toner may be observed by this image analysis by using a brightness difference (contrast) between the epoxy resin used in embedding and the binder resin of the toner. A long axis length of the release agent domain in the toner and an aspect ratio thereof are determined based on the observed image.

20 Subsequently, a centroid position of the release agent domain extracted by using a brightness difference (contrast) between the binder resin and the release agent is obtained as follows. x coordinates of the centroids are values obtained 25 by dividing summation of respective  $x_i$  coordinate values by n, and y coordinates of the centroids are values obtained by dividing summation of respective  $y_i$  coordinate values by n, when the number of pixels in an area of the extracted toner or the extracted release agent domain is set as n, xy coordinates of each pixel are set as  $x_i$  and  $y_i$  ( $i=1, 2, \dots, n$ ).

30 An angle formed by a tangent line passing a tangent point of a circumference of a circle centered at a centroid of the release agent domain and inscribed in an outer edge of the toner particle and the outer edge, and a line which passes the centroid of the release agent domain and extends in the long axis direction of the release agent domain is determined from the determined centroid and the observed image.

35 In the exemplary embodiment, a percentage of the toner particles including the specific release agent domains in the entire toner particles is preferably equal to or greater than 30 number %, more preferably equal to or greater than 40 number %, and even more preferably equal to or greater than 50 number %, from a viewpoint of peeling properties of a fixed image from a fixing member. It is more preferable that 40 the percentage of the toner particles including the specific release agent domains in the entire toner particles is equal to or greater than 30 number %, from a viewpoint of peeling properties of a fixed image from a fixing member.

45 In the exemplary embodiment, the number of toner particles to be evaluated when calculating the percentage of the toner particles including the specific release agent domains in the entire toner particles is 100 or more.

The adjustment of the percentage of the toner particles including the specific release agent domains in the entire toner particles may be performed by adjusting the position of the release agent in the process of forming the toner particle and causing the release agent domain to grow by heating.

## External Additive

50 Examples of the external additive include inorganic particles. Examples of the inorganic particles include  $\text{SiO}_2$ ,  $\text{TiO}_2$ ,  $\text{Al}_2\text{O}_3$ ,  $\text{CuO}$ ,  $\text{ZnO}$ ,  $\text{SnO}_2$ ,  $\text{CeO}_2$ ,  $\text{Fe}_2\text{O}_3$ ,  $\text{MgO}$ ,  $\text{BaO}$ ,  $\text{CaO}$ ,  $\text{K}_2\text{O}$ ,  $\text{Na}_2\text{O}$ ,  $\text{ZrO}_2$ ,  $\text{CaO} \cdot \text{SiO}_2$ ,  $\text{K}_2\text{O} \cdot (\text{TiO}_2)_n$ ,  $\text{Al}_2\text{O}_3 \cdot 2\text{SiO}_2$ ,  $\text{CaCO}_3$ ,  $\text{MgCO}_3$ ,  $\text{BaSO}_4$ , and  $\text{MgSO}_4$ .

55 Surfaces of the inorganic particles as an external additive are preferably subjected to a hydrophobizing treatment. The hydrophobizing treatment is performed by, for example,

dipping the inorganic particles in a hydrophobizing agent. The hydrophobizing agent is not particularly limited and examples thereof include a silane coupling agent, silicone oil, a titanate coupling agent, and an aluminum coupling agent. These may be used alone or in combination of two or more kinds thereof.

Generally, the amount of the hydrophobizing agent is, for example, from 1 part by weight to 10 parts by weight with respect to 100 parts by weight of the inorganic particles.

Examples of the external additive also include resin particles (resin particles such as polystyrene, PMMA, and melamine resin particles) and a cleaning aid (e.g., metal salt of higher fatty acid represented by zinc stearate, and fluorine-based polymer particles).

The amount of the external additive externally added is, for example, preferably from 0.01% by weight to 5% by weight, and more preferably from 0.01% by weight to 2.0% by weight with respect to the toner particles.

#### Toner Preparing Method

Next, a method of preparing a toner according to this exemplary embodiment will be described.

The toner according to this exemplary embodiment is obtained by externally adding an external additive to toner particles after preparing of the toner particles.

The toner particles may be prepared using any of a dry preparing method (e.g., kneading and pulverizing method) and a wet preparing method (e.g., aggregation and coalescence method, suspension and polymerization method, and dissolution and suspension method). The toner particle preparing method is not particularly limited to these preparing methods, and a known preparing method is employed.

Among these, the toner particles are preferably obtained by an aggregation and coalescence method.

Specifically, for example, when the toner particles are manufactured by an aggregation and coalescence method, the toner particles are manufactured through the processes of: preparing a resin particle dispersion in which resin particles as a binder resin are dispersed (resin particle dispersion preparation process); aggregating each of the resin particles (if necessary, other particles) in the resin particle dispersion (if necessary, in a dispersion after mixing with other particle dispersions) to form aggregated particles (aggregated particle forming process); and heating the aggregated particle dispersion in which the aggregated particles are dispersed, to coalesce the aggregated particles, thereby forming toner particles (coalescence process).

Hereinafter, the respective processes will be described in detail.

In the following description, a method of obtaining toner particle containing a colorant and a release agent will be described, but the colorant is used if necessary. Additives other than the colorant may be used.

#### Resin Particle Dispersion Preparation Process

First, for example, a colorant particle dispersion in which colorant particles are dispersed and a release agent particle dispersion in which release agent particles are dispersed are prepared together with a resin particle dispersion in which resin particles as a binder resin are dispersed.

Herein, the resin particle dispersion is prepared by, for example, dispersing resin particles by a surfactant in a dispersion medium.

Examples of the dispersion medium used for the resin particle dispersion include aqueous mediums.

Examples of the aqueous mediums include water such as distilled water and ion exchange water, and alcohols. These may be used alone or in combination of two or more kinds thereof.

Examples of the surfactant include anionic surfactants such as sulfuric ester salt, sulfonate, phosphate, and soap anionic surfactants; cationic surfactants such as amine salt and quaternary ammonium salt cationic surfactants; and nonionic surfactants such as polyethylene glycol, alkyl phenol ethylene oxide adduct, and polyol nonionic surfactants. Among these, anionic surfactants and cationic surfactants are particularly used. Nonionic surfactants may be used in combination with anionic surfactants or cationic surfactants.

The surfactants may be used alone or in combination of two or more kinds thereof.

Regarding the resin particle dispersion, as a method of dispersing the resin particles in the dispersion medium, a common dispersing method using, for example, a rotary shearing-type homogenizer, or a ball mill, a sand mill, or a Dyne mill having media is exemplified. Depending on the kind of the resin particles, resin particles may be dispersed in the resin particle dispersion using, for example, a phase inversion emulsification method.

The phase inversion emulsification method includes: dissolving a resin to be dispersed in a hydrophobic organic solvent in which the resin is soluble; conducting neutralization by adding a base to an organic continuous phase (O phase); and converting the resin (so-called phase inversion) from W/O to O/W by putting an aqueous medium (W phase) to form a discontinuous phase, thereby dispersing the resin as particles in the aqueous medium.

A volume average particle diameter of the resin particles dispersed in the resin particle dispersion is, for example, preferably from 0.01  $\mu\text{m}$  to 1  $\mu\text{m}$ , more preferably from 0.08  $\mu\text{m}$  to 0.8  $\mu\text{m}$ , and even more preferably from 0.1  $\mu\text{m}$  to 0.6  $\mu\text{m}$ .

Regarding the volume average particle diameter of the resin particles, a cumulative distribution by volume is drawn from the side of the smallest diameter with respect to particle size ranges (channels) divided using the particle size distribution obtained by the measurement with a laser diffraction-type particle size distribution measuring device (for example, LA-700 manufactured by Horiba, Ltd.), and a particle diameter when the cumulative percentage becomes 50% with respect to the entire particles is measured as a volume average particle diameter D50v. The volume average particle diameter of the particles in other dispersions is also measured in the same manner.

The content of the resin particles contained in the resin particle dispersion is, for example, preferably from 5% by weight to 50% by weight, and more preferably from 10% by weight to 40% by weight.

For example, the colorant particle dispersion and the release agent particle dispersion are also prepared in the same manner as in the case of the resin particle dispersion. That is, the particles in the resin particle dispersion are the same as the colorant particles dispersed in the colorant particle dispersion and the release agent particles dispersed in the release agent particle dispersion, in terms of the volume average particle diameter, the dispersion medium, the dispersing method, and the content of the particles.

#### Aggregated Particle Forming Process

Next, the colorant particle dispersion and the release agent particle dispersion are mixed together with the resin particle dispersion.

The resin particles, the colorant particles, the release agent particles are heterogeneously aggregated in the mixed dispersion, thereby forming aggregated particles having a

## 15

diameter near a target toner particle diameter and including the resin particles, colorant particles, and the release agent particles.

Specifically, for example, an aggregating agent is added to the mixed dispersion and a pH of the mixed dispersion is adjusted to acidity (for example, the pH is from 2 to 5). If necessary, a dispersion stabilizer is added. Then, the mixed dispersion is heated at a temperature of the glass transition temperature of the resin particles (specifically, for example, from a temperature 30° C. lower than the glass transition temperature of the resin particles to a temperature 10° C. lower than the glass transition temperature) to aggregate the particles dispersed in the mixed dispersion, thereby forming the aggregated particles.

In the aggregated particle forming process, for example, the aggregating agent may be added at room temperature (for example, 25° C.) under stirring of the mixed dispersion using a rotary shearing-type homogenizer, the pH of the mixed dispersion may be adjusted to acidic (for example, the pH is from 2 to 5), a dispersion stabilizer may be added if necessary, and the heating may then be performed.

Examples of the aggregating agent include a surfactant having an opposite polarity to the polarity of the surfactant used as the dispersing agent to be added to the mixed dispersion, such as inorganic metal salts and di- or higher-valent metal complexes. Particularly, when a metal complex is used as the aggregating agent, the amount of the surfactant used is reduced and charging characteristics are improved.

If necessary, an additive may be used which forms a complex or a similar bond with the metal ions of the aggregating agent. A chelating agent is preferably used as the additive.

Examples of the inorganic metal salt include a metal salt such as calcium chloride, calcium nitrate, barium chloride, magnesium chloride, zinc chloride, aluminum chloride, and aluminum sulfate, and inorganic metal salt polymer such as polyaluminum chloride, polyaluminum hydroxide, and calcium polysulfide.

A water-soluble chelating agent may be used as the chelating agent. Examples of the chelating agent include oxycarboxylic acids such as tartaric acid, citric acid, and gluconic acid, iminodiacetic acid (IDA), nitrilotriacetic acid (NTA), and ethylenediaminetetraacetic acid (EDTA).

An addition amount of the chelating agent is, for example, preferably in a range of from 0.01 parts by weight to 5.0 parts by weight, and more preferably in a range of from 0.1 parts by weight to less than 3.0 parts by weight relative to 100 parts by weight of the resin particles.

## Coalescence Process

Next, the aggregated particle dispersion in which the aggregated particles are dispersed is heated at, for example, a temperature that is equal to or higher than the glass transition temperature of the resin particles (for example, a temperature that is higher than the glass transition temperature of the resin particles by 10° C. to 30° C.) to coalesce the aggregated particles and form toner particles.

The toner particles are obtained through the above-described processes.

The toner particles may be prepared through the processes of: after the aggregated particle dispersion in which the aggregated particles are dispersed is obtained, further mixing the aggregated particle dispersion with a resin particle dispersion in which resin particles are dispersed to perform aggregation so that the resin particles further adhere to the surfaces of the aggregated particles, thereby forming second aggregated particles; and coalescing the second aggregated particles by heating the second aggregated particle disper-

## 16

sion in which the second aggregated particles are dispersed, and thereby forming toner particles having a core/shell structure.

When preparing toner particles having a core/shell structure, in the process of forming the second aggregated particles, the aggregated particle dispersion, the resin particle dispersion in which the resin particles are dispersed, the release agent particle dispersion in which release agent particles are dispersed, and the inorganic mineral may be further mixed with each other to perform aggregation so that the resin particles, the release agent particles, and the inorganic mineral further adhere to the surfaces of the aggregated particles.

In addition, a toner particle including a core particle, a first shell layer coated on the core particle, and a second shell layer coated on the first shell layer may be prepared. In this case, toner particles may be prepared through the processes of: after obtaining the aggregated particle dispersion in which the aggregated particles are dispersed, further mixing the aggregated particle dispersion, a resin particle dispersion in which resin particles are dispersed, and a release agent particle dispersion in which release agent particles are dispersed with each other to perform aggregation so that the resin particles and the release agent particles further adhere to the surfaces of the aggregated particles, thereby forming third aggregated particles; further mixing the third aggregated particle dispersion, the resin particle dispersion in which the resin particles are dispersed, and the inorganic mineral with each other to perform aggregation so that the resin particles and the inorganic mineral further adhere to the surfaces of the third aggregated particles, thereby forming fourth aggregated particles; and coalescing the fourth aggregated particles by heating a fourth aggregated particle dispersion in which the fourth aggregated particles are dispersed, and thereby forming toner particles having a core/first shell/second shell structure. In the process of forming the third aggregated particles described above, the inorganic mineral may be further incorporated (that is, the inorganic mineral may be further incorporated in both processes of forming the third aggregated particles and forming the fourth aggregated particles). The inorganic mineral mixed in each process described above may be mixed as an inorganic mineral dispersion by preparing the inorganic mineral dispersion in which the inorganic mineral is dispersed.

For controlling of arrangement of the release agent domains, a method of temporarily performing cooling after forming the toner particles having a core/first shell/second shell structure, and then increasing the temperature to a melting temperature of the release agent is used. By performing cooling and increasing the temperature to a melting temperature of the release agent in a state where the release agent particles contained in the first shell is interposed between binder resin particles contained in the core and binder resin particles contained in the second shell, the release agent domains slowly grow in the first shell and a growth direction of the domains is easily oriented to a shell layer direction. As a result, it is possible to control the growth direction of the release agent domains and it is easy to satisfy the specific release agent domains.

After the coalescence process is ended, toner particles formed in a solution are subjected to a well-known washing process, a well-known solid-liquid separation process, a well-known drying process, and thereby dried toner particles are obtained.

Regarding the washing process, replacing washing using ion exchanged water may preferably be sufficiently performed for charging property. The solid-liquid separation

process is not particularly limited, but suction filtration, pressure filtration, or the like may preferably be performed for productivity. The drying process is not particularly limited, but freeze drying, flash jet drying, fluidized drying, vibrating fluidized drying, and the like may preferably be performed for productivity.

The toner according to the exemplary embodiment is prepared, for example, by adding an external additive to the obtained toner particles in a dried state, and performing mixing. The mixing may be performed, for example, by using a V blender, a HENSCHEL mixer, a LÖDIGE mixer, or the like. Furthermore, if necessary, coarse toner particles may be removed using a vibration sieving machine, a wind classifier, or the like.

#### Electrostatic Charge Image Developer

An electrostatic charge image developer according to this exemplary embodiment includes at least the toner according to this exemplary embodiment.

The electrostatic charge image developer according to this exemplary embodiment may be a single-component developer including only the toner according to this exemplary embodiment, or a two-component developer obtained by mixing the toner with a carrier.

The carrier is not particularly limited, and known carriers are exemplified. Examples of the carrier include a coated carrier in which surfaces of cores formed of a magnetic powder are coated with a coating resin; a magnetic powder dispersion-type carrier in which a magnetic powder is dispersed and blended in a matrix resin; and a resin impregnation-type carrier in which a porous magnetic powder is impregnated with a resin.

The magnetic powder dispersion-type carrier and the resin impregnation-type carrier may be carriers in which constituent particles of the carrier are cores and coated with a coating resin.

Examples of the magnetic powder include magnetic metals such as iron, nickel, and cobalt, and magnetic oxides such as ferrite and magnetite.

Examples of the coating resin and the matrix resin include polyethylene, polypropylene, polystyrene, polyvinyl acetate, polyvinyl alcohol, polyvinyl butyral, polyvinyl chloride, polyvinyl ether, polyvinyl ketone, a vinyl chloride-vinyl acetate copolymer, a styrene-acrylic ester copolymer, a straight silicone resin configured to include an organosiloxane bond or a modified product thereof, a fluororesin, a polyester, polycarbonate, a phenol resin, and an epoxy resin.

The coating resin and the matrix resin may contain other additives such as a conductive particles.

Examples of the conductive particles include particles of metals such as gold, silver, and copper, carbon black particles, titanium oxide particles, zinc oxide particles, tin oxide particles, barium sulfate particles, aluminum borate particles, and potassium titanate particles.

Here, a coating method using a coating layer forming solution in which a coating resin, and if necessary, various additives are dissolved or dispersed in an appropriate solvent is used to coat the surface of a core with the coating resin. The solvent is not particularly limited, and may be selected in consideration of the coating resin to be used, coating suitability, and the like.

Specific examples of the resin coating method include a dipping method of dipping cores in a coating layer forming solution, a spraying method of spraying a coating layer forming solution to surfaces of cores, a fluid bed method of spraying a coating layer forming solution in a state in which cores are allowed to float by flowing air, and a kneader-coater method in which cores of a carrier and a coating layer

forming solution are mixed with each other in a kneader-coater and the solvent is removed.

The mixing ratio (weight ratio) between the toner and the carrier in the two-component developer is preferably from 1:100 to 30:100, and more preferably from 3:100 to 20:100 (toner:carrier).

#### Image Forming Apparatus/Image Forming Method

An image forming apparatus and an image forming method according to this exemplary embodiment will be described.

The image forming apparatus according to this exemplary embodiment is provided with an image holding member, a charging unit that charges a surface of the image holding member, an electrostatic charge image forming unit that forms an electrostatic charge image on a charged surface of the image holding member, a developing unit that contains an electrostatic charge image developer and develops the electrostatic charge image formed on the surface of the image holding member with the electrostatic charge image developer to form a toner image, a transfer unit that transfers the toner image formed on the surface of the image holding member onto a surface of a recording medium, and a fixing unit that fixes the toner image transferred onto the surface of the recording medium. As the electrostatic charge image developer, the electrostatic charge image developer according to this exemplary embodiment is applied.

In the image forming apparatus according to this exemplary embodiment, an image forming method (image forming method according to this exemplary embodiment) including a charging process of charging a surface of an image holding member, an electrostatic charge image forming process of forming an electrostatic charge image on a charged surface of the image holding member, a developing process of developing the electrostatic charge image formed on the surface of the image holding member with the electrostatic charge image developer according to this exemplary embodiment to form a toner image, a transfer process of transferring the toner image formed on the surface of the image holding member onto a surface of a recording medium, and a fixing process of fixing the toner image transferred onto the surface of the recording medium is performed.

As the image forming apparatus according to this exemplary embodiment, a known image forming apparatus is applied, such as a direct transfer-type apparatus that directly transfers a toner image formed on a surface of an image holding member onto a recording medium; an intermediate transfer-type apparatus that primarily transfers a toner image formed on a surface of an image holding member onto a surface of an intermediate transfer member, and secondarily transfers the toner image transferred onto the surface of the intermediate transfer member onto a surface of a recording medium; an apparatus that is provided with a cleaning unit that cleans a surface of an image holding member after transfer of a toner image and before charging; or an apparatus that is provided with an erasing unit that irradiates, after transfer of a toner image and before charging, a surface of an image holding member with erasing light for erasing.

In the case of an intermediate transfer-type apparatus, a transfer unit has, for example, an intermediate transfer member having a surface onto which a toner image is to be transferred, a primary transfer unit that primarily transfers a toner image formed on a surface of an image holding member onto the surface of the intermediate transfer member, and a secondary transfer unit that secondarily transfers the toner image transferred onto the surface of the intermediate transfer member onto a surface of a recording medium.

In the image forming apparatus according to this exemplary embodiment, for example, a part including the developing unit may have a cartridge structure (process cartridge) that is detachable from the image forming apparatus. As the process cartridge, for example, a process cartridge that stores the electrostatic charge image developer according to this exemplary embodiment and is provided with a developing unit is preferably used.

Hereinafter, an example of the image forming apparatus according to this exemplary embodiment will be shown. However, this image forming apparatus is not limited thereto. Major parts shown in the drawing will be described, but descriptions of other parts will be omitted.

FIG. 2 is a schematic diagram showing a configuration of the image forming apparatus according to this exemplary embodiment.

The image forming apparatus shown in FIG. 2 is provided with first to fourth electrophotographic image forming units **10Y**, **10M**, **10C**, and **10K** (image forming units) that output yellow (Y), magenta (M), cyan (C), and black (K) images based on color-separated image data, respectively. These image forming units (hereinafter, may be simply referred to as "units") **10Y**, **10M**, **10C**, and **10K** are arranged side by side at predetermined intervals in a horizontal direction. These units **10Y**, **10M**, **10C**, and **10K** may be process cartridges that are detachable from the image forming apparatus.

An intermediate transfer belt **20** as an intermediate transfer member is installed above the units **10Y**, **10M**, **10C**, and **10K** in the drawing to extend through the units. The intermediate transfer belt **20** is wound on a driving roll **22** and a support roll **24** contacting the inner surface of the intermediate transfer belt **20**, which are disposed to be separated from each other on the left and right sides in the drawing, and travels in a direction toward the fourth unit **10K** from the first unit **10Y**. The support roll **24** is pressed in a direction in which it departs from the driving roll **22** by a spring or the like (not shown), and a tension is given to the intermediate transfer belt **20** wound on both of the rolls. In addition, an intermediate transfer member cleaning device **30** opposed to the driving roll **22** is provided on a surface of the intermediate transfer belt **20** on the image holding member side.

Developing devices (developing units) **4Y**, **4M**, **4C**, and **4K** of the units **10Y**, **10M**, **10C**, and **10K** are supplied with toner including four color toner, that is, a yellow toner, a magenta toner, a cyan toner, and a black toner stored in toner cartridges **8Y**, **8M**, **8C**, and **8K**, respectively.

The first to fourth units **10Y**, **10M**, **10C**, and **10K** have the same configuration, and accordingly, only the first unit **10Y** that is disposed on the upstream side in a traveling direction of the intermediate transfer belt to form a yellow image will be representatively described herein. The same parts as in the first unit **10Y** will be denoted by the reference numerals with magenta (M), cyan (C), and black (K) added instead of yellow (Y), and descriptions of the second to fourth units **10M**, **10C**, and **10K** will be omitted.

The first unit **10Y** has a photoreceptor **1Y** acting as an image holding member. Around the photoreceptor **1Y**, a charging roll (an example of the charging unit) **2Y** that charges a surface of the photoreceptor **1Y** to a predetermined potential, an exposure device (an example of the electrostatic charge image forming unit) **3** that exposes the charged surface with laser beams **3Y** based on a color-separated image signal to form an electrostatic charge image, a developing device (an example of the developing unit) **4Y** that supplies a charged toner to the electrostatic charge image to develop the electrostatic charge image, a primary transfer

roll (an example of the primary transfer unit) **5Y** that transfers the developed toner image onto the intermediate transfer belt **20**, and a photoreceptor cleaning device (an example of the cleaning unit) **6Y** that removes the toner remaining on the surface of the photoreceptor **1Y** after primary transfer, are arranged in sequence.

The primary transfer roll **5Y** is disposed inside the intermediate transfer belt **20** to be provided at a position opposed to the photoreceptor **1Y**. Furthermore, bias supplies (not shown) that apply a primary transfer bias are connected to the primary transfer rolls **5Y**, **5M**, **5C**, and **5K**, respectively. Each bias supply changes a transfer bias that is applied to each primary transfer roll under the control of a controller (not shown).

Hereinafter, an operation of forming a yellow image in the first unit **10Y** will be described.

First, before the operation, the surface of the photoreceptor **1Y** is charged to a potential of -600 V to -800 V by the charging roll **2Y**.

The photoreceptor **1Y** is formed by laminating a photosensitive layer on a conductive substrate (for example, volume resistivity at 20° C.:  $1 \times 10^{-6} \Omega\text{cm}$  or less). The photosensitive layer typically has high resistance (that is about the same as the resistance of a general resin), but has properties in which when laser beams **3Y** are applied, the specific resistance of a part irradiated with the laser beams changes. Accordingly, the laser beams **3Y** are output to the charged surface of the photoreceptor **1Y** via the exposure device **3** in accordance with image data for yellow sent from the controller (not shown). The laser beams **3Y** are applied to the photosensitive layer on the surface of the photoreceptor **1Y**, whereby an electrostatic charge image of a yellow image pattern is formed on the surface of the photoreceptor **1Y**.

The electrostatic charge image is an image that is formed on the surface of the photoreceptor **1Y** by charging, and is a so-called negative electrostatic charge image, that is formed by applying laser beams **3Y** to the photosensitive layer so that the specific resistance of the irradiated part is lowered to cause charges to flow on the surface of the photoreceptor **1Y**, while charges stay on a part to which the laser beams **3Y** are not applied.

The electrostatic charge image formed on the photoreceptor **1Y** is rotated up to a predetermined developing position with the travelling of the photoreceptor **1Y**. The electrostatic charge image on the photoreceptor **1Y** is visualized (developed) as a toner image at the developing position by the developing device **4Y**.

The developing device **4Y** stores, for example, an electrostatic charge image developer including at least a yellow toner and a carrier. The yellow toner is frictionally charged by being agitated in the developing device **4Y** to have a charge with the same polarity (negative polarity) as the charge that is on the photoreceptor **1Y**, and is thus held on the developer roll (an example of the developer holding member). By allowing the surface of the photoreceptor **1Y** to pass through the developing device **4Y**, the yellow toner electrostatically adheres to the erased electrostatic charge image part on the surface of the photoreceptor **1Y**, whereby the electrostatic charge image is developed with the yellow toner. Next, the photoreceptor **1Y** having the yellow toner image formed thereon continuously travels at a predetermined rate and the toner image developed on the photoreceptor **1Y** is transported to a predetermined primary transfer position.

When the yellow toner image on the photoreceptor **1Y** is transported to the primary transfer position, a primary trans-

fer bias is applied to the primary transfer roll 5Y and an electrostatic force toward the primary transfer roll 5Y from the photoreceptor 1Y acts on the toner image, whereby the toner image on the photoreceptor 1Y is transferred onto the intermediate transfer belt 20. The transfer bias applied at this time has the opposite polarity (+) to the toner polarity (-), and, for example, is controlled to +10  $\mu$ A in the first unit 10Y by the controller (not shown).

On the other hand, the toner remaining on the photoreceptor 1Y is removed and collected by the photoreceptor cleaning device 6Y.

The primary transfer biases that are applied to the primary transfer rolls 5M, 5C, and 5K of the second unit 10M and the subsequent units are also controlled in the same manner as in the case of the first unit.

In this manner, the intermediate transfer belt 20 onto which the yellow toner image is transferred in the first unit 10Y is sequentially transported through the second to fourth units 10M, 10C, and 10K, and the toner images of respective colors are multiply-transferred in a superimposed manner.

The intermediate transfer belt 20 onto which the four color toner images have been multiply-transferred through the first to fourth units reaches a secondary transfer part that is composed of the intermediate transfer belt 20, the support roll 24 contacting the inner surface of the intermediate transfer belt, and a secondary transfer roll (an example of the secondary transfer unit) 26 disposed on the image holding surface side of the intermediate transfer belt 20. Meanwhile, a recording sheet (an example of the recording medium) P is supplied to a gap between the secondary transfer roll 26 and the intermediate transfer belt 20, that are brought into contact with each other, via a supply mechanism at a predetermined timing, and a secondary transfer bias is applied to the support roll 24. The transfer bias applied at this time has the same polarity (-) as the toner polarity (-), and an electrostatic force toward the recording sheet P from the intermediate transfer belt 20 acts on the toner image, whereby the toner image on the intermediate transfer belt 20 is transferred onto the recording sheet P. In this case, the secondary transfer bias is determined depending on the resistance detected by a resistance detector (not shown) that detects the resistance of the secondary transfer part, and is voltage-controlled.

Thereafter, the recording sheet P is fed to a pressure-contacting part (nip part) between a pair of fixing rolls in a fixing device (an example of the fixing unit) 28 so that the toner image is fixed to the recording sheet P, whereby a fixed image is formed.

Examples of the recording sheet P onto which a toner image is transferred include plain paper that is used in electrophotographic copiers, printers, and the like. As a recording medium, an OHP sheet is also exemplified other than the recording sheet P.

The surface of the recording sheet P is preferably smooth in order to further improve smoothness of the image surface after fixing. For example, coating paper obtained by coating a surface of plain paper with a resin or the like, art paper for printing, and the like are preferably used.

The recording sheet P on which the fixing of the color image is completed is discharged toward a discharge part, and a series of the color image forming operations end.

#### Process Cartridge/Toner Cartridge

A process cartridge according to this exemplary embodiment will be described.

The process cartridge according to this exemplary embodiment is provided with a developing unit that stores the electrostatic charge image developer according to this

exemplary embodiment and develops an electrostatic charge image formed on a surface of an image holding member with the electrostatic charge image developer to form a toner image, and is detachable from an image forming apparatus.

The process cartridge according to this exemplary embodiment is not limited to the above-described configuration, and may be configured to include a developing device, and if necessary, at least one selected from other units such as an image holding member, a charging unit, an electrostatic charge image forming unit, and a transfer unit.

Hereinafter, an example of the process cartridge according to this exemplary embodiment will be shown. However, this process cartridge is not limited thereto. Major parts shown in the drawing will be described, but descriptions of other parts will be omitted.

FIG. 3 is a schematic diagram showing a configuration of the process cartridge according to this exemplary embodiment.

A process cartridge 200 shown in FIG. 3 is formed as a cartridge having a configuration in which a photoreceptor 107 (an example of the image holding member), a charging roll 108 (an example of the charging unit), a developing device 111 (an example of the developing unit), and a photoreceptor cleaning device 113 (an example of the cleaning unit), which are provided around the photoreceptor 107, are integrally combined and held by the use of, for example, a housing 117 provided with a mounting rail 116 and an opening 118 for exposure.

In FIG. 3, the reference numeral 109 represents an exposure device (an example of the electrostatic charge image forming unit), the reference numeral 112 represents a transfer device (an example of the transfer unit), the reference numeral 115 represents a fixing device (an example of the fixing unit), and the reference numeral 300 represents a recording sheet (an example of the recording medium).

Next, a toner cartridge according to this exemplary embodiment will be described.

The toner cartridge according to this exemplary embodiment stores the toner according to this exemplary embodiment and is detachable from an image forming apparatus. The toner cartridge stores a toner in a storing portion for replenishment for being supplied to the developing unit provided in the image forming apparatus.

The image forming apparatus shown in FIG. 2 has such a configuration that the toner cartridges 8Y, 8M, 8C, and 8K are detachable therefrom, and the developing devices 4Y, 4M, 4C, and 4K are connected to the toner cartridges corresponding to the respective developing devices (colors) via toner supply tubes (not shown), respectively. In addition, when the toner stored in the toner cartridge runs low, the toner cartridge is replaced.

#### EXAMPLES

Hereinafter, the exemplary embodiment will be described more specifically using examples and comparative examples, but the exemplary embodiment is not limited to these examples. Unless specifically noted, "parts" and "%" are based on weight.

| Preparation of Polyester Resin (1)              |           |
|-------------------------------------------------|-----------|
| 2 mol adduct of ethylene oxide of bisphenol A:  | 114 parts |
| 2 mol adduct of propylene oxide of bisphenol A: | 84 parts  |

23

-continued

## Preparation of Polyester Resin (1)

|                              |            |
|------------------------------|------------|
| Dimethylester terephthalate: | 75 parts   |
| Dodeceny succinic acid:      | 19.5 parts |
| Trimellitic acid:            | 7.5 parts  |

The above components are put into a 5-liter flask including a stirrer, a nitrogen gas introducing tube, a temperature sensor, and a rectifier, heated to a temperature of 190° C. over 1 hour, and stirring is performed in a reaction system, and 3.0 parts of dibutyl tin oxide is put therein. The temperature is increased to 240° C. from 190° C. over 6 hours while distilling away generated water, a dehydration condensation reaction is further continued at 240° C. for 2 hours, and thus, a polyester resin (1) is synthesized.

Regarding the obtained polyester resin (1), a glass transition temperature is 54° C., an acid value is 15.3 mgKOH/g, a weight average molecular weight is 58,000, and a number average molecular weight is 5,600.

## Preparation of Polyester Resin Particle Dispersion (1)

|                                                                           |           |
|---------------------------------------------------------------------------|-----------|
| Polyester resin (1) (Mw: 58,000):                                         | 144 parts |
| Isopropyl acrylamide (manufactured by Kohjin Film & Chemicals Co., Ltd.): | 16 parts  |
| Ethyl acetate:                                                            | 233 parts |
| Sodium hydroxide aqueous solution (0.3 N):                                | 0.1 parts |

The above components are put in a 1000-mL separable flask, heated at 70° C., and stirred with a Three-One Motor (manufactured by Shinto Scientific Co., Ltd.) to prepare a resin mixed liquid. 373 parts of the ion exchange water is slowly added therein while further stirring the resin mixed liquid, to thereby perform phase inversion emulsification, and the solvent thereof is removed to obtain a polyester resin particle dispersion (1) (solid content concentration: 30%). A volume average particle diameter of the resin particles in the dispersion is 160 nm.

## Preparation of release agent particle dispersion (1)

|                                                                                              |           |
|----------------------------------------------------------------------------------------------|-----------|
| Fischer Tropsch wax (melting temperature of 92° C., manufactured by Nippon Seiro Co., Ltd.): | 180 parts |
| Anionic surfactant (NEOGEN R manufactured by Dai-Ichi Kogyo Seiyaku Co., Ltd.):              | 4.5 parts |
| Ion exchange water:                                                                          | 410 parts |

The above components are heated at 110° C. and dispersed using a homogenizer (ULTRA TURRAX T50 manufactured by IKA Japan, K.K.). After that, the mixture is subjected to dispersion treatment with MANTON-GAULIN high pressure homogenizer (manufactured by Gaulin Co., Ltd.), to thereby disperse release agent particles having a volume average particle diameter of 0.24  $\mu\text{m}$ , and the concentration is adjusted using ion exchange water, and thus, a release agent particle dispersion (1) in which solid concentration of the release agent particles is 30.0% by weight is prepared.

## Preparation of Release Agent Particle Dispersion (2)

A release agent particle dispersion (2) in which solid concentration of the release agent particles is 30.0% by

24

weight is prepared in the same manner as in the preparation of the release agent particle dispersion (1), except for using paraffin wax HNP0190 (melting temperature of 85° C., manufactured by Nippon Seiro Co., Ltd.) instead of Fischer Tropsch wax used in the preparation of the release agent particle dispersion (1).

## Preparation of Release Agent Particle Dispersion (3)

A release agent particle dispersion (3) in which solid concentration of the release agent particles is 30.0% by weight is prepared in the same manner as in the preparation of the release agent particle dispersion (1), except for using polyethylene wax POLYWAX725 (melting temperature of 104° C., manufactured by Baker Petrolite Corporation) instead of Fischer Tropsch wax used in the preparation of the release agent particle dispersion (1).

## Preparation of Colorant Particle Dispersion

|                                                                                                                                              |           |
|----------------------------------------------------------------------------------------------------------------------------------------------|-----------|
| C.I. Pigment Red 238 (FUJI FAST CARMINE 580 manufactured by Fuji Pigment Co., Ltd.):                                                         | 250 parts |
| Anionic surfactant (NEOGEN SC manufactured by Dai-Ichi Kogyo Seiyaku Co., Ltd.): (60% of active ingredient, 8% with respect to the colorant) | 33 parts  |
| Ion exchange water:                                                                                                                          | 750 parts |

280 parts of ion exchange water and 33 parts of anionic surfactant are put in a stainless steel vessel having such a size that a height of a liquid surface when all of the above components are put therein is approximately  $\frac{1}{3}$  of the height of the vessel, the surfactant is sufficiently dissolved, the 35 pigments are all put therein, the resultant material is stirred using a stirrer until no unmet pigments remain, and sufficiently defoamed. The remaining ion exchange water is added thereto after the defoaming, the resultant material is dispersed by using a homogenizer (ULTRA TURRAX T50 40 manufactured by IKA Japan, K.K.) at 5,000 rpm for 10 minutes, is stirred and defoamed using the stirrer for 24 hours. After the defoaming, the resultant material is dispersed again by using the homogenizer at 6,000 rpm for 10 minutes, is stirred and defoamed using the stirrer for 24 45 hours. Then, the dispersion is dispersed by using a high pressure impact type dispersing machine ULTIMIZER (HJP30006 manufactured by Sugino Machine, Ltd.) at a pressure of 240 MPa. The dispersion is performed with about 25 passes based on the conversion from the total 50 introduction amount and processing capacity of the device. The obtained dispersion is allowed to stand for 72 hours to remove precipitates, ion exchange water is added to provide a solid content concentration of 20%. A volume average particle diameter D50 of the particles in the colorant particle dispersion is 135 nm.

## Preparation of Inorganic Mineral Dispersion (1)

|                                                                                     |           |
|-------------------------------------------------------------------------------------|-----------|
| Smectite (bentonite product "ODOSORUBU" manufactured by Kurozaki Hakudo Kogyo KK.): | 40 parts  |
| Anionic surfactant (NEOGEN R manufactured by Dai-Ichi Kogyo Seiyaku Co., Ltd.):     | 4.0 parts |
| Ion exchange water:                                                                 | 396 parts |

65 The above components are dispersed using a homogenizer (ULTRA TURRAX T50 manufactured by IKA Japan, K.K.) at room temperature. After that, the mixture is subjected to

25

dispersion treatment with MANTON-GAULIN high pressure homogenizer (manufactured by Gaulin Co., Ltd.), inorganic mineral particles having a volume average particle diameter of 0.50  $\mu\text{m}$  are dispersed therein, and the concentration is adjusted using ion exchange water, to thereby prepare an inorganic mineral dispersion (1) in which solid concentration of the inorganic mineral is 10.0% by weight.

#### Preparation of Inorganic Mineral Dispersion (2)

An inorganic mineral dispersion (2) in which solid concentration of the inorganic mineral is 10.0% by weight is prepared in the same manner as in the preparation of the inorganic mineral dispersion (1), except for using kaolinite (product name: STATINTONE No. 5 manufactured by Takehara Kagaku Kogyo Co., Ltd.) instead of smectite used in the preparation of the inorganic mineral dispersion (1).

#### Example 1

| Preparation of Toner (1)                                                                 |           |
|------------------------------------------------------------------------------------------|-----------|
| Ion exchange water:                                                                      | 215 parts |
| Polyester resin particle dispersion (1):                                                 | 203 parts |
| Colorant particle dispersion:<br>(solid content of 20%)                                  | 20 parts  |
| Anionic surfactant:<br>(NEOGEN RK manufactured by Dai-Ichi Kogyo Seiyaku Co., Ltd., 20%) | 2.8 parts |

The above components are put in a 3-liter reaction vessel including a thermometer, a pH meter, and a stirrer, and maintained at 30° C. and a stirring rotation rate of 150 rpm for 30 minutes, while controlling a temperature with a mantle heater from the outside. After that, 0.3 N nitric acid aqueous solution is added to thereby adjust the pH in the aggregation process to 3.0.

A polyaluminium chloride aqueous solution in which 0.7 parts of polyaluminium chloride is dissolved in 7 parts of ion exchange water is added to the mixture, while dispersing with a homogenizer (ULTRA TURRAX T50 manufactured by IKA Japan, K.K.). After that, the temperature is increased to 50° C. while stirring, a particle diameter is measured using a COULTER MULTISIZER II (aperture diameter: 50  $\mu\text{m}$ , manufactured by Beckman Coulter, Inc.), and a volume average particle diameter is adjusted to 5.0  $\mu\text{m}$ . Then, a mixed solution of 30 parts of the polyester resin particle dispersion (1) and 15 parts of the release agent particle dispersion (1) is added. After 30 minutes, 45 parts of the polyester resin particle dispersion (1) and 20 parts of the inorganic mineral dispersion (1) as the inorganic mineral are further added, so that the resin particles and the inorganic minerals are attached (shell structure) to the surfaces of the aggregated particles.

After adding 20 parts of 10% by weight nitrilotriacetic acid (NTA) metal salt solution (CHELEST 70 manufactured by Chelest Corporation), the pH is adjusted to 9.0 using 1 N sodium hydroxide aqueous solution. Then, the temperature is increased to 90° C. by setting a rate of temperature increase at 0.05° C./min, the temperature is maintained at 90° C. for 3 hours, and then the mixture is cooled. After that, in order to cause the release agent domains to grow, the resultant material is heated to 92° C. which is a temperature equal to or higher than the melting temperature of the release agent and maintained for 30 minutes, slowly cooled to 30° C. at a rate of 2° C./min, and filtered to obtain coarse toner

26

particles. This is further re-dispersed in ion exchange water, and filtered, the cycle of the re-dispersion and filtration is repeated to perform washing until electric conductivity of the filtrate becomes equal to or smaller than 20  $\mu\text{S}/\text{cm}$ , and the resultant material is subjected to vacuum-drying in an oven at 40° C. for 5 hours, and thus, toner particles (1) are obtained.

10 1.5 parts by weight of hydrophobic silica (RY50 manufactured by Nippon Aerosil Co. Ltd.) and 1.0 part by weight of hydrophobic titanium oxide (T805 manufactured by Nippon Aerosil Co. Ltd.) are mixed with respect to 100 parts by weight of the obtained toner particles (1) using a sample mill at 10,000 rpm for 30 seconds. After that, the mixture is 15 sieved by a vibration sieving device having an aperture of 45  $\mu\text{m}$ , and thus, a toner (1) is prepared. A volume average particle diameter of the obtained toner (1) is 6.1  $\mu\text{m}$ .

#### Example 2

##### Preparation of Toner (2)

Toner particles (2) and a toner (2) are obtained in the same manner as in the preparation of the toner (1), except for changing the kind of the inorganic mineral to the inorganic mineral dispersion (2) according to Table 1.

#### Example 3

##### Preparation of Toner (3)

30 After performing the aggregation process in the same manner as in the preparation of the toner (1), the temperature is increased to 50° C., a particle diameter is measured using COULTER MULTISIZER II, and a volume average particle diameter is adjusted to 5.0  $\mu\text{m}$ . Then, a toner (3) is prepared in the same manner as in the preparation of the toner (1), except for changing the addition of the mixed solution of 30 parts of the polyester resin particle dispersion (1) and 15 parts of the release agent particle dispersion (1) in the preparation of the toner (1) to addition of a mixed solution of 35 parts of the polyester resin particle dispersion (1) and 10 parts of the release agent particle dispersion (1).

#### Example 4

##### Preparation of Toner (4)

35 After performing the aggregation process in the same manner as in the preparation of the toner (1), the temperature is increased to 50° C., a particle diameter is measured using COULTER MULTISIZER II, and a volume average particle diameter is adjusted to 5.0  $\mu\text{m}$ . Then, a toner (4) is prepared in the same manner as in the preparation of the toner (1), except for changing the addition of the mixed solution of 30 parts of the polyester resin particle dispersion (1) and 15 parts of the release agent particle dispersion (1) in the preparation of the toner (1) to addition of a mixed solution of 25 parts of the polyester resin particle dispersion (1) and 20 parts of the release agent particle dispersion (1).

#### Example 5

##### Preparation of Toner (5)

40 45 50 55 60 65 The release agent particle dispersion (1) used in the preparation of the toner (1) is changed to the release agent particle dispersion (2). A toner (5) is prepared in the same

manner as in the preparation of the toner (1), except for changing the heating to 92° C. which is a temperature equal to or higher than the melting temperature of the release agent to the heating to 85° C. which is a temperature equal to or higher than the melting temperature of the release agent after performing the aggregation process in the same manner as in the preparation of the toner (1).

#### Example 6

##### Preparation of Toner (6)

The release agent particle dispersion (1) used in the preparation of the toner (1) is changed to the release agent particle dispersion (3). A toner (6) is prepared in the same manner as in the preparation of the toner (1), except for changing the heating to 92° C. which is a temperature equal to or higher than the melting temperature of the release agent to the heating to 104° C. which is a temperature equal to or higher than the melting temperature of the release agent after performing the aggregation process in the same manner as in the preparation of the toner (1).

#### Example 7

##### Preparation of Toner (7)

After performing the aggregation process in the same manner as in the preparation of the toner (1), the temperature is increased to 50° C., a particle diameter is measured using COULTER MULTISIZER II, and a volume average particle diameter is adjusted to 5.0 µm. Then, a mixed solution of 30 parts of the polyester resin particle dispersion (1) and 15 parts of the release agent particle dispersion (1) is added. A toner (7) is prepared in the same manner as in the preparation of the toner (1), except for changing the addition of 45 parts of the polyester resin particle dispersion (1) and 20 parts of the inorganic mineral dispersion (1) as the inorganic mineral which is performed 30 minutes after the previous addition, to addition of 75 parts of the polyester resin particle dispersion (1), 15 parts of the release agent particle dispersion (1), and 20 parts of the inorganic mineral dispersion (1).

#### Example 8

##### Preparation of Toner (8)

|                                                                                       |           |
|---------------------------------------------------------------------------------------|-----------|
| Ion exchange water:                                                                   | 215 parts |
| Polyester resin particle dispersion (1):                                              | 237 parts |
| Colorant particle dispersion:                                                         | 20 parts  |
| (solid content of 2096)                                                               |           |
| Anionic surfactant (NEOGEN RK manufactured by Dai-Ichi Kogyo Seiyaku Co., Ltd., 20%): | 2.8 parts |

The above components are put in a 3-liter reaction vessel including a thermometer, a pH meter, and a stirrer, and maintained at 30° C. and a stirring rotation rate of 150 rpm for 30 minutes, while controlling a temperature with a mantle heater from the outside. After that, 0.3 N nitric acid aqueous solution is added to thereby adjust the pH in the aggregation process to 3.0.

A polyaluminium chloride aqueous solution in which 0.7 parts of polyaluminium chloride is dissolved in 7 parts of ion exchange water is added to the mixture, while dispersing with a homogenizer (ULTRA TURRAX T50 manufactured

by IKA Japan, K.K.). After that, the temperature is increased to 50° C. while stirring, a particle diameter is measured using a COULTER MULTISIZER II (aperture diameter: 50 µm, manufactured by Beckman Coulter, Inc.), and a volume average particle diameter is adjusted to 5.0 µm. Then, a mixed solution of 27 parts of the polyester resin particle dispersion (1) and 15 parts of the release agent particle dispersion (1) is added. After 30 minutes, 35 parts of the polyester resin particle dispersion (1) and 20 parts of the inorganic mineral dispersion (1) as the inorganic mineral are further added, so that the resin particles and the inorganic minerals are attached (shell structure) to the surfaces of the aggregated particles. Then, a toner (8) is prepared in the same manner as in the preparation of the toner (1).

#### Comparative Example 1

##### Preparation of Toner (C1)

|                                                                                       |           |
|---------------------------------------------------------------------------------------|-----------|
| Ion exchange water:                                                                   | 215 parts |
| Polyester resin particle dispersion (1):                                              | 170 parts |
| Colorant particle dispersion:                                                         | 20 parts  |
| Release agent particle dispersion (1):                                                | 33 parts  |
| Anionic surfactant (NEOGEN RK manufactured by Dai-Tchi Kogyo Seiyaku Co., Ltd., 20%): | 2.8 parts |

The above components are put in a 3-liter reaction vessel including a thermometer, a pH meter, and a stirrer, and maintained at 30° C. and a stirring rotation rate of 150 rpm for 30 minutes, while controlling a temperature with a mantle heater from the outside. After that, 0.3 N nitric acid aqueous solution is added to thereby adjust the pH in the aggregation process to 3.0.

A polyaluminium chloride aqueous solution in which 0.7 parts of polyaluminium chloride is dissolved in 7 parts of ion exchange water is added to the mixture, while dispersing with a homogenizer (ULTRA TURRAX T50 manufactured by IKA Japan, K.K.). After that, the temperature is increased to 50° C. while stirring, a particle diameter is measured using a COULTER MULTISIZER II (aperture diameter: 50 µm, manufactured by Beckman Coulter, Inc.), and a volume average particle diameter is adjusted to 5.0 µm. Then, 116 parts of the polyester resin particle dispersion (1) is added, so that the resin particles are attached (shell structure) to the surfaces of the aggregated particles.

After adding 20 parts of 10% nitrilotriacetic acid (NTA) metal salt solution (CHELEST 70 manufactured by Chelest Corporation), pH is adjusted to 9.0 using 1 N sodium hydroxide aqueous solution. Then, the temperature is increased to 90° C. by setting a rate of temperature increase at 0.05° C./min, the temperature is maintained at 90° C. for 3 hours, and then the mixture is cooled and filtered to obtain coarse toner particles. This is further re-dispersed in ion exchange water, and filtered, the cycle of the re-dispersion and filtration is repeated to perform washing until electric conductivity of the filtrate becomes equal to or smaller than 20 µS/cm, and the resultant material is subjected to vacuum-drying in an oven at 40° C. for 5 hours, and toner particles (C1) are obtained.

1.5 parts of hydrophobic silica (RY50 manufactured by Nippon Aerosil Co. Ltd.) and 1.0 part of hydrophobic titanium oxide (T805 manufactured by Nippon Aerosil Co. Ltd.) are mixed with respect to 100 parts of the obtained toner particles (C1) using a sample mill at 10,000 rpm for 30 seconds. After that, the mixture is sieved by a vibration sieving device having an aperture of 45 µm, and a toner (C1)

29

is prepared. A volume average particle diameter of the obtained toner (C1) is 6.1  $\mu\text{m}$ .

## Comparative Example 2

| Preparation of Toner (C2)                                                             |           |
|---------------------------------------------------------------------------------------|-----------|
| Ion exchange water:                                                                   | 215 parts |
| Polyester resin particle dispersion (1):                                              | 203 parts |
| Colorant particle dispersion:                                                         | 20 parts  |
| Anionic surfactant (NEOGEN RK manufactured by Dai-Ichi Kogyo Seiyaku Co., Ltd., 20%): | 2.8 parts |

The above components are put in a 3-liter reaction vessel including a thermometer, a pH meter, and a stirrer, and maintained at 30° C. and a stirring rotation rate of 150 rpm for 30 minutes, while controlling a temperature with a mantle heater from the outside. After that, 0.3 N nitric acid aqueous solution is added to thereby adjust the pH in the aggregation process to 3.0.

A polyaluminium chloride aqueous solution in which 0.7 parts of polyaluminium chloride is dissolved in 7 parts of ion exchange water is added to the mixture, while dispersing with a homogenizer (ULTRA TURRAX T50 manufactured by IKA Japan, K.K.). After that, the temperature is increased to 50° C. while stirring, a particle diameter is measured using a COULTER MULTISIZER II (aperture diameter: 50  $\mu\text{m}$ , manufactured by Beckman Coulter, Inc.), and a volume average particle diameter is adjusted to 5.0  $\mu\text{m}$ . Then, 45 parts of the polyester resin particle dispersion (1) is added. After 30 minutes, a mixed solution of 57 parts of the polyester resin particle dispersion (1) and 15 parts of the release agent particle dispersion (1) is added, so that the release agent particles and the resin particles are attached (shell structure) to the surfaces of the aggregated particles.

After adding 20 parts of 10% by weight nitrilotriacetic acid (NTA) metal salt solution (CHELEST 70 manufactured by Chelest Corporation), pH is adjusted to 9.0 using 1 N sodium hydroxide aqueous solution. Then, the temperature is increased to 90° C. by setting a rate of temperature increase at 0.05° C./min, the temperature is maintained at 90° C. for 3 hours, and then the mixture is cooled and filtered to obtain coarse toner particles. This is further re-dispersed in ion exchange water and filtered, the cycle of the re-dispersion and filtration is repeated to perform washing until electric conductivity of the filtrate becomes equal to or smaller than 20  $\mu\text{S}/\text{cm}$ , and the resultant material is subjected to vacuum-drying in an oven at 40° C. for 5 hours, and thus, toner particles (C2) are obtained.

1.5 parts by weight of hydrophobic silica (RY50 manufactured by Nippon Aerosil Co. Ltd.) and 1.0 part by weight of hydrophobic titanium oxide (T805 manufactured by Nippon Aerosil Co. Ltd.) are mixed with respect to 100 parts by weight of the obtained toner particles (C2) using a sample mill at 10,000 rpm for 30 seconds. After that, the mixture is sieved by a vibration sieving device having an aperture of 45  $\mu\text{m}$ , and a toner (C2) is prepared. A volume average particle diameter of the obtained toner (C2) is 6.1  $\mu\text{m}$ .

## Comparative Example 3

| Preparation of Toner (C3)                |           |
|------------------------------------------|-----------|
| Ion exchange water:                      | 215 parts |
| Polyester resin particle dispersion (1): | 170 parts |

30

-continued

| Preparation of Toner (C3) |                                                                   |           |
|---------------------------|-------------------------------------------------------------------|-----------|
| 5                         | Colorant particle dispersion:                                     | 20 parts  |
|                           | Release agent particle dispersion (1):                            | 33 parts  |
|                           | Anionic surfactant:                                               | 2.8 parts |
|                           | (NEOGEN RK manufactured by Dai-Ichi Kogyo Seiyaku Co., Ltd., 20%) |           |

10 The above components are put in a 3-liter reaction vessel including a thermometer, a pH meter, and a stirrer, and maintained at 30° C. and a stirring rotation rate of 150 rpm for 30 minutes, while controlling a temperature with a mantle heater from the outside. After that, 0.3 N nitric acid aqueous solution is added to thereby adjust the pH in the aggregation process to 3.0.

15 A polyaluminium chloride aqueous solution in which 0.7 parts of polyaluminium chloride is dissolved in 7 parts of ion exchange water is added to the mixture, while dispersing with a homogenizer (ULTRA TURRAX T50 manufactured by IKA Japan, K.K.). After that, the temperature is increased to 50° C. while stirring, a particle diameter is measured using a COULER MULTISIZER II (aperture diameter: 50  $\mu\text{m}$ , manufactured by Beckman Coulter, Inc.), and a volume average particle diameter is adjusted to 5.0  $\mu\text{m}$ . Then, 110 parts of the polyester resin particle dispersion (1) and 20 parts of the inorganic mineral dispersion (1) are added, so that the resin particles and the inorganic mineral are attached (shell structure) to the surfaces of the aggregated particles.

20 After adding 20 parts of 10% nitrilotriacetic acid (NTA) metal salt solution (CHELEST 70 manufactured by Chelest Corporation), pH is adjusted to 9.0 using 1 N sodium hydroxide aqueous solution. Then, the temperature is increased to 90° C. by setting a rate of temperature increase at 0.05° C./min, the temperature is maintained at 90° C. for 3 hours, and then the mixture is cooled and filtered to obtain coarse toner particles. This is further re-dispersed in ion exchange water and filtered, the cycle of the re-dispersion and filtration is repeated to perform washing until electric conductivity of the filtrate becomes equal to or smaller than 20  $\mu\text{S}/\text{cm}$ , and the resultant material is subjected to vacuum-drying in an oven at 40° C. for 5 hours, and toner particles (C3) are obtained.

25 30 35 40 45 50 55 500 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9

## 31

First, a solution obtained by diluting carbon black in toluene is added to a perfluoroacrylate copolymer and the resultant is dispersed by a sand mill. The above components except for ferrite particles are dispersed therein with a stirrer for 10 minutes and a coating layer forming solution is prepared. Then, the coating layer forming solution and the ferrite particles are put in a vacuum degassing type kneader, and stirred at 60°C. for 30 minutes, toluene is distilled away under the reduced pressure, and thus, a resin coating layer is formed to obtain a carrier.

## Preparation of Developer

36 parts of the toner (1) and 414 parts of the carrier are put in a 2-liter V-blender, stirred for 20 minutes, and sieved with a sieve having an aperture of 212 µm, and a developer (1) is prepared.

Developers (2) to (C3) are prepared in the same manner as in the preparation of the developer (1), except for using the toner prepared in each example instead of the toner (1).

## Evaluation

## Evaluation of Image Deletion

“DOCUCENTRE COLOR 400CP” manufactured by Fuji Xerox Co., Ltd. is prepared as an image forming apparatus, and a developing device is filled with each developer obtained.

Images based on The Imaging Society of Japan Test Chart No. 8 (image density of 5%) are continuously printed on

## 32

Ltd. so as to print an unfixed image up to an edge of the paper is prepared, a developing device is filled with each developer obtained, and a toner cartridge is filled with each toner obtained. Then, a full solid image having a toner amount of 0.8 mg/cm<sup>2</sup> is formed on an SP sheet (paper thickness of 81 µm and paper weight of 60 g/m<sup>2</sup> manufactured by Fuji Xerox Co., Ltd.), and 100 sheets are continuously printed by setting a fixing temperature to 180°C. and a process speed to 220 mm/sec. The following evaluations are performed with respect to the obtained image on the 100th sheet. The evaluation is performed in the environment of a temperature of 25°C. and humidity of 60%. A state of the edge of the sheet is observed with respect to obtained image on the 100th sheet and evaluated with the following criteria.

## Evaluation Criteria

A: peeling failure has not occurred and the state of the edge of the sheet is also excellent

B: peeling failure has not occurred and the edge of the sheet is slightly curled

C: slight peeling failure has occurred and the edge of the image is slightly disturbed

D: peeling failure has clearly occurred

The presence ratio of the inorganic mineral, the presence ratio of the release agent, and the percentage of the specific release agent domains are measured by the methods described above.

TABLE 1

| Kind       | Inorganic mineral |                |             | Release agent |                |             |                           |            |   |
|------------|-------------------|----------------|-------------|---------------|----------------|-------------|---------------------------|------------|---|
|            | surface %         | Presence ratio |             | surface %     | Presence ratio |             | of specific release agent | Percentage |   |
|            |                   | 400 nm from    | 300 nm from |               | 400 nm from    | 300 nm from |                           | Evaluation |   |
| Ex. 1      | Smectite          | 95             | 85          | (1)           | 90             | 20          | 70                        | A          | A |
| Ex. 2      | Kaolinite         | 95             | 80          | (1)           | 90             | 15          | 70                        | A          | A |
| Ex. 3      | Smectite          | 95             | 80          | (1)           | 95             | 20          | 60                        | A          | B |
| Ex. 4      | Smectite          | 95             | 85          | (1)           | 80             | 15          | 70                        | A          | A |
| Ex. 5      | Smectite          | 95             | 80          | (2)           | 85             | 17          | 60                        | A          | A |
| Ex. 6      | Smectite          | 95             | 85          | (3)           | 80             | 15          | 10                        | A          | B |
| Ex. 7      | Smectite          | 95             | 65          | (1)           | 95             | 65          | 70                        | B          | B |
| Ex. 8      | Smectite          | 95             | 95          | (1)           | 95             | 80          | 70                        | B          | B |
| Com. Ex. 1 | None              | 0              | 0           | (1)           | 10             | 0           | 10                        | C          | D |
| Com. Ex. 2 | None              | 0              | 0           | (1)           | 90             | 65          | 70                        | C          | A |
| Com. Ex. 3 | Smectite          | 100            | 70          | (1)           | 10             | 0           | 10                        | A          | D |

10,000 A4-sized sheets using the image forming apparatus in a high temperature and high humidity environment (in an environment of temperature of 32°C. and humidity of 90 RH %). Then, solid images having image density of 90% and a toner amount of 5.0 g/m<sup>2</sup> are printed on 100 A4-sized sheets and the images on the first 10 printed sheets are visually observed.

## Evaluation Criteria

A: no image deletion is observed in any images

B: image deletion is observed in some images but it is in an acceptable level

C: image deletion which is visually clearly recognized is observed in some images and is in an unacceptable level

## Evaluation of Peeling Properties

An image forming apparatus which forms an image for evaluation, an apparatus obtained by modifying “DOCUCENTRE-IV C4700P” manufactured by Fuji Xerox Co.,

50 In Table 1, the “presence ratio” in a column of the inorganic mineral shows a percentage of the inorganic mineral present in a portion within 400 nm or 300 nm from the surface of the toner particle with respect to the entire inorganic mineral.

55 The “presence ratio” in a column of the release agent shows a percentage of the release agent present in a portion within 400 nm or 300 nm from the surface of the toner particle with respect to the entire release agent.

The “percentage of the specific release agent domains” means a percentage of the toner particles including the specific release agent domains in the entire toner particles.

60 From the above results, it is found that results of evaluation of “image deletion” are excellent in the examples, compared to the comparative examples. Accordingly, it is found that occurrence of image deletion is prevented in the examples, compared to the comparative examples.

In addition, it is found that "peeling properties" are excellent in the examples, compared to the comparative examples.

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention be defined by the following claims and their equivalents.

What is claimed is:

1. An electrostatic charge image developing toner comprising:

a toner particle containing a binder resin, a release agent, and an inorganic mineral,

wherein 80% or more of the entire release agent is present in a portion within 400 nm from a surface of the toner particle, and

80% or more of the entire inorganic mineral is present in a portion within 400 nm from the surface of the toner particle.

2. The electrostatic charge image developing toner according to claim 1,

wherein 20% or less of the entire release agent is present in a portion within 300 nm from the surface of the toner particle, and

80% or more of the entire inorganic mineral is present in a portion within 300 nm from the surface of the toner particle.

3. The electrostatic charge image developing toner according to claim 1,

wherein the release agent forms release agent domains satisfying Conditions (1) to (4):

Condition (1): a length of the release agent domain in a long axis direction is from 300 nm to 1200 nm;

Condition (2): a ratio between a length of the release agent domain in a long axis direction and a length thereof in a short axis direction (length in a long axis direction/length in a short axis direction) is from 3.0 to 15.0;

Condition (3): an angle formed by a tangent line passing a tangent point of a circumference of a circle centered at a centroid of the release agent domain and inscribed in an outer edge of the toner particle and the outer edge, and a line which passes the centroid of the release agent domain and extends in the long axis direction of the release agent domain is from 0° to 45°; and

Condition (4): a ratio between a circle equivalent diameter of the toner particle and a distance A between the centroid of the release agent domain and the tangent point (distance A/circle equivalent diameter) is from 0.03 to 0.25.

4. The electrostatic charge image developing toner according to claim 1,

wherein the inorganic mineral is a layered clay mineral.

5. The electrostatic charge image developing toner according to claim 4,

wherein the layered clay mineral is selected from the group consisting of kaolinite, smectite, illite, mica, vermiculite, talc, pyrophyllite, and chlorite.

6. The electrostatic charge image developing toner according to claim 1,

wherein a content of the inorganic mineral is from 1% by weight to 10% by weight with respect to the entire toner particles.

7. The electrostatic charge image developing toner according to claim 1, wherein a weight ratio of the inorganic mineral to the release agent is in a range of from 1:1 to 1:15.

8. An electrostatic charge image developer, comprising a carrier and the electrostatic charge image developing toner according to claim 1.

9. A toner cartridge which is detachable from an image forming apparatus comprising:

a storing portion that stores the electrostatic charge image developing toner according to claim 1.

\* \* \* \* \*